

No. 723,717.

PATENTED MAR. 24, 1903.

J. D. NICHOLSON.

ELECTRIC CONDUCTOR.

APPLICATION FILED AUG. 17, 1900.

NO MODEL.



WITNESSES:

*John D. Nicholson*, INVENTOR

*Emilly S. Anderson*  
*Finis D. Morris.*

BY  
*Tho. J. M. Tighe*  
ATTORNEY

# UNITED STATES PATENT OFFICE.

JOHN D. NICHOLSON, OF PITTSBURG, PENNSYLVANIA, ASSIGNOR TO THE PITTSBURGH REDUCTION COMPANY, OF PITTSBURG, PENNSYLVANIA, A CORPORATION OF PENNSYLVANIA.

## ELECTRIC CONDUCTOR.

SPECIFICATION forming part of Letters Patent No. 723,717, dated March 24, 1903.

Application filed August 17, 1900. Serial No. 27,196. (No model.)

*To all whom it may concern:*

Be it known that I, JOHN D. NICHOLSON, a citizen of the United States, and a resident of Pittsburgh, in the county of Allegheny and

5 State of Pennsylvania, have invented a certain new and useful Improvement in Electrical Conductors, of which the following is a specification.

This invention relates to a novel electrical conductor or wire; and it consists in a wire drawn or rolled from a compound ingot made of two metals, one being copper and the other aluminium, substantially as hereinafter fully described and claimed.

15 In the drawing which forms part of this specification the figure is a transverse section of my compound wire.

Some of the more pertinent physical characteristics of aluminium and copper are as 20 follows:

|                                                        | Aluminium.            | Copper.               |
|--------------------------------------------------------|-----------------------|-----------------------|
| Specific gravity                                       | 2.68                  | 8.93                  |
| Relative specific gravity                              | 1                     | 3.33                  |
| Relative electric conductivity                         | 61                    | 98                    |
| Tensile strength per square inch                       | 24,000 to 55,000 lbs. | 30,000 to 60,000 lbs. |
| Relative sectional area for same electric conductivity | 150                   | 100                   |
| 30 Relative weight for same electric conductivity      | 47.77                 | 100                   |

The two metals readily fuse together to form alloys of more or less value in the mechanical arts; but the important electric characteristics then no longer exist. The electric conductivity, for example, diminishes rapidly with the addition of copper, while the tensile strength may increase greatly.

40 I have found that a wire can be readily drawn from a compound ingot composed of the two metals poured or formed separately, in some cases the core being of copper and the shell of aluminium, in other cases the reverse.

45 In such a wire each metal preserves its own characteristics and both metals partake in the increase of tensile strength due to the operation of drawing. The conductivity of either

remains intact. By duly proportioning the two metals the resultant strength, conductivity, sectional area, or weight may be brought to any desired standard.

I prefer to make the compound wire with a copper core and aluminium shell on account of the greatly-reduced liability to corrosion. 55 In coupling such wires or making branch connections the difficulty ordinarily found in soldering aluminium is not serious, as the copper part of the conductor can be readily soldered without seriously raising the resistance 60 of the joint.

The particular method of forming the compound ingot may vary, as that is not of the essence of my present invention. A simple way is by casting first a core of copper, it having the higher melting-point, and then while this is at or near the melting-point of aluminium casting the shell of the latter around such copper core, or the operation may be reversed as to positions, the first cast, of copper, 70 being the shell and the cast of aluminium being the core, or in some cases the hollow and solid ingots may be separately formed and consolidated by hydraulic or other pressure applied before or after cooling or while the 75 core is cold and the shell still heated.

In referring to either of the two component parts of my new conductor I wish to say that they are supposed to be substantially pure; but the presence of slight admixtures of phosphorus or other well-known deoxidizing reagents is not objectionable, provided the individual characteristics of the two metals are substantially preserved.

I claim as my invention—

5 A compound electrical conductor composed of a core and a shell of different metals drawn into wire, one metal being aluminium and the other copper.

Signed at the city of Belfast, Ireland, this 90 9th day of July, 1900.

JOHN D. NICHOLSON.

Witnesses:

JOHN M. QUADE,  
BERNARD PEEKE.